

April 5, 1949.

D. J. BUCKLEY ET AL

2,466,300

CONTINUOUS PLASTICIZATION PROCESS

Filed April 28, 1945

7 Sheets-Sheet 1



FIG. - 1

Donald J. Buckley  
Allen L. Chaney Inventors

By R. Young Attorney

April 5, 1949.

D. J. BUCKLEY ET AL

2,466,300

CONTINUOUS PLASTICIZATION PROCESS

Filed April 28, 1945

7 Sheets-Sheet 2

EFFECT OF MERCAPTAN CONCENTRATION AND  
ORIGINAL MOONEY VISCOSITY AT MILL TEMPERATURE 100°F.



FIG. 2

Donald J. Buckley Inventor  
Allen L. Chaney Inventor

By P. Young Attorney

April 5, 1949.

D. J. BUCKLEY ET AL

2,466,300

CONTINUOUS PLASTICIZATION PROCESS

Filed April 28, 1945

7 Sheets-Sheet 3

EFFECT OF MERCAPTAN CONCENTRATION AND  
ORIGINAL MOONEY VISCOSITY AT MILL TEMPERATURE 150°F.



FIG. - 3

Donald J. Buckley  
Allen L. Chaney Inventors

By P. H. Young Attorney

April 5, 1949.

D. J. BUCKLEY ET AL

2,466,300

CONTINUOUS PLASTICIZATION PROCESS

Filed April 28, 1945

7 Sheets-Sheet 4

EFFECT OF MERCAPTAN CONCENTRATION AND  
ORIGINAL MOONEY VISCOSITY AT MILL TEMPERATURE 200°F.



FIG. - 4

Donald J. Buckley Inventors  
Allen L. Chorley

By John Young Attorney

April 5, 1949.

D. J. BUCKLEY ET AL

2,466,300

CONTINUOUS PLASTICIZATION PROCESS

Filed April 28, 1945

7 Sheets-Sheet 5

EFFECT OF MERCAPTAN CONCENTRATION AND  
ORIGINAL MOONEY VISCOSITY AT MILL TEMPERATURE 250°F.



PERCENT CONCENTRATION OF MERCAPTAN

FIG. - 5

Donald J. Buckley Inventors  
Allen L. Chaney Inventors

By P. H. Young Attorney

April 5, 1949.

D. J. BUCKLEY ET AL

2,466,300

CONTINUOUS PLASTICIZATION PROCESS

Filed April 28, 1945

7 Sheets-Sheet 6

EFFECT OF MERCAPTAN CONCENTRATION AND  
ORIGINAL MOONEY VISCOSITY AT MILL TEMPERATURE 300°F.



PERCENT CONCENTRATION OF MERCAPTAN

FIG.-6

Donald J. Buckley Inventor  
Allen L. Chaney Inventor

By Ph. Young Attorney

April 5, 1949.

D. J. BUCKLEY ET AL

2,466,300

CONTINUOUS PLASTICIZATION PROCESS

Filed April 28, 1945.

7 Sheets-Sheet 7



Donald J. Buckley  
Allen L. Chaney Inventors

By P. Young Attorney

## UNITED STATES PATENT OFFICE

2,466,300

## CONTINUOUS PLASTICIZATION PROCESS

Donald J. Buckley, Plainfield, N. J., and Allen L. Chaney, Baton Rouge, La., assignors to Standard Oil Development Company, a corporation of Delaware

Application April 28, 1945, Serial No. 590,842

5 Claims. (CL 266—30.8)

1

This invention relates to a process for working up rubber-like polymeric materials and relates more especially to means for the plasticizing of such polymers.

It has been found possible to interpolymerize an isoolefin such as isobutylene with one or more polyolefins such as butadiene, isoprene, piperylene, dimethyl butadiene, and the like, at temperatures ranging from 0° C. or —40° C. to —160° C. by the application thereto of a dissolved Friedel-Crafts catalyst. These polymers have comparatively very high molecular weights and comparatively low iodine numbers; and they are reactive with sulfur in a curing reaction which has some points of similarity to the vulcanization of rubber to yield extremely valuable rubber-like synthetic bodies. However, difficulty is encountered in the milling and processing of many of these polymers, especially those of very high molecular weight. The polymers of moderately high molecular weights are readily milled, cure readily and yield good rubber-like bodies but they do not have the maximum in tensile strength. Polymers having very high molecular weights yield cured bodies having exceedingly good tensile strength, elongation, abrasion resistance, flexure resistance and other valuable properties.

In the production of these polymers, conditions are sometimes such that the average molecular weight of the product is higher than is consistent with good processability in practical application. Current rubber manufacturing practice has indicated that good processability is obtained at a value of 40-55 as measured on the Mooney viscometer in a 1½ minute test at 100° C. It is, therefore, an advantage to have a system whereby high molecular weight product could be reduced in viscosity value so that it would meet processability requirements.

The production of high molecular weight polymers is, however, not without certain advantages for if the polymerization operation can be carried out without the necessity of bringing the Mooney viscosity value of the product down into the range of 40-55, then the process would be smoother and production rates higher. Furthermore, those conditions in the polymerization operation which produce high molecular weight polymers are conducive to less fouling of the reactor surfaces, and the minimizing of overflow plugs between the reactor and the recovery system. This condition tends to increase the number of on-catalyst hours for a given polymerization cycle.

In the preparation of these polymers the reactor liquor and product are dumped into a flash

2

tank for the purpose of removing unreacted monomers and diluent. The polymer is dispersed in the water in this tank in the form of an aqueous slurry. The water in the flash tank is maintained at approximately 150° F. Considering the fact that the polymer is thermoplastic, it is easy to visualize why the low molecular weight products tend to agglomerate in this tank, and why the high molecular weight products form discrete particles in the aqueous medium. The satisfactory operation of this flash tank and the water slurry system in general is dependent on the formation of small discrete particles in this phase of the process. In addition to this, the fine discrete particles formed from the high molecular weight product are easily dried in the subsequent tunnel dryer equipment while the agglomerated particles resulting from the low molecular weight product are a constant source of unsatisfactory operation in the drying step.

In the polymer drying section of the process it has been definitely established that high molecular weight products dry more satisfactorily than do the low molecular weight products. Even though low molecular weight products may come to the drying section in the form of discrete particles, the greater thermoplasticity of these polymers causes them to fuse in the dryer and prevents the proper throughput of air required for satisfactory drying. Considerable plant experimentation on this point indicates that only those polymers which have a Mooney viscosity value in excess of 60 will dry satisfactorily in the standard tunnel dryer equipment.

Furthermore, the plasticization of a high molecular weight polymer down to the range of 40-55 Mooney viscosity provides a narrower molecular weight distribution than is obtained by polymerizing a product to fall within this viscosity range originally. Narrow ranges of molecular weight distribution provide the optimum in vulcanizate quality.

It is thus readily seen that considerable advantage is obtained if high molecular weight polymers are produced in the polymerization process and then continuously plasticized to fall into the required viscosity range. It has been found that the polymers can be plasticized if they are milled in the presence of a small quantity of an aryl type mercaptan at a sufficiently high temperature. As an example of this, a polymer, possessing an original Mooney viscosity value of 81, was milled at a temperature of 300° F. for a period of 10 minutes in the presence of

a range of concentrations of naphthyl-beta-mercaptan with the following results.

| Sample   | Concentration, Percent Naphthyl-beta-mercaptan | Effective Concentration, Percent Naphthyl-beta Mercaptan | Mooney Viscosity $1\frac{1}{2}$ at $100^{\circ}\text{C}$ . |
|----------|------------------------------------------------|----------------------------------------------------------|------------------------------------------------------------|
| Original |                                                |                                                          | 81                                                         |
| Sample 1 | 0.00                                           | 0.00                                                     | 80                                                         |
| Sample 2 | 0.10                                           | 0.030                                                    | 63                                                         |
| Sample 3 | 0.25                                           | 0.075                                                    | 47                                                         |
| Sample 4 | 0.50                                           | 0.150                                                    | 40                                                         |
| Sample 5 | 0.75                                           | 0.225                                                    | 36                                                         |
| Sample 6 | 1.00                                           | 0.30                                                     | 33                                                         |

The plasticization achieved in this experiment is proportional to the mercaptan concentration employed. This proportionality decreases as the concentration of mercaptan increases. Concentrations of mercaptan of 0.25 percent (0.075 percent effective) or less are sufficient to achieve the desired Mooney viscosity reduction.

The present invention provides a highly efficient continuous process for improving the processing characteristics of these polymers through the use of aryl mercaptans as plasticizing agents, with minimum sacrifices in the desirable physical properties of the cured vulcanizate subsequently obtained.

Thus the process of the invention covers the preparation of a polymer having a molecular weight much higher than that desired and the continuous plasticization of this high polymer to the desired molecular weight by means of train operations employing any suitable plasticizing agent. The product of the invention is a rubber-like polymer which is readily processed before curing, and shows a high tensile strength and other valuable properties after curing. Other objects and details of the invention will be apparent from the following description.

In practicing the invention, the polymeric material is preferably prepared from a mixture of a major proportion of an isolefin which is preferably isobutylene, but may be other isolefins such as 2-methyl butene-1, or 2 methyl pentene-1, or the like; together with a minor proportion of a polyolefin such as butadiene or isoprene or piperylene, or dimethyl butadiene, or myrcene, or dimethylallyl, or the like, the preferred polyolefins having from 4 to 12 or 14 carbon atoms per molecule. The olefinic material is cooled to temperatures ranging from  $0^{\circ}\text{C}$ . to  $-100^{\circ}\text{C}$ . or even as low as  $-164^{\circ}\text{C}$ ., and the polymerization is conducted by the application to the cold olefinic material of a Friedel-Crafts catalyst dissolved in a low-freezing, non-complex-forming solvent such as ethyl or methyl chloride or carbon disulfide or the like.

The Friedel-Crafts catalyst may be any of the Friedel-Crafts catalysts disclosed by N. O. Caloway in his article on the "Friedel-Crafts synthesis" appearing in the issue of "Chemical Reviews," published for the American Chemical Society at Baltimore in 1935, in volume XVII, No. 3, the article beginning on page 327, the list being particularly well shown on page 375. For the solvent, substantially any of the lower mono- or polyalkyl halides having freezing points below about  $-10^{\circ}\text{C}$ . may be used. The Friedel-Crafts catalyst is dissolved in the solvent and mixed with the cold olefinic material, preferably by application in the form of a spray to the surface of the rapidly stirred cold olefinic mixture. The polymerization thereupon proceeds rapidly

to yield a solid polymer having a relatively very high molecular weight.

These polymers are conveniently evaluated by their Mooney viscosity. This test, as described in Industrial and Engineering Chemistry, Analytical Edition, vol. 2, page 147 (1934), consists in shearing the polymer between the roughened surfaces of a disc shaped rotor and the upper and lower halves of a stator chamber. Two

samples of the polymer, each two inches square and  $\frac{1}{4}$  to  $\frac{3}{8}$  inch thick, are used, one piece being placed above the rotor and the other beneath it. A pressure of 30 to 60 kg./sq. cm. (400 to 800 lbs./sq. inch) is exerted on the polymer by means of plungers.

The rotor is connected through a vertical spindle, worm gear and horizontal floating shaft to a synchronous A. C. motor. The motion of the floating shaft is indicated on a dial gauge which reads zero when the plastometer is empty. The platens surrounding the stator chamber are maintained at  $212^{\circ}\text{F}$ . The sample is allowed to warm up for one minute after being inserted and the platens closed. A gauge reading is obtained after one and one-half minute. This gauge reading is proportional to the viscosity and is reported as the Mooney viscosity.

Another useful method for determining the plasticity is described by Williams in the Industrial and Engineering Chemistry, vol. 16, page 362 (1924). In this test a spherical sample of polymer of 2 cc. volume is placed between two parallel plates and a load of 5 kg. is applied to it for three minutes. The resulting thickness of the sample is called the plasticity number or simply the Williams plasticity. The sample is then immediately removed and allowed to cool for one minute at room temperature. The increase in thickness of the deformed pellet on cooling is called the recovery figure.

After the completion of the polymerization reaction, the solid polymer is separated from the liquid residue of the reaction mixture and brought up to room temperature. It may be washed and purified on the mill to remove traces

of catalyst and residual traces of unpolymerized material. However, any other method for removing residual catalyst and unreacted monomers may be employed as desired. It is then compounded with a suitable softening agent.

Suitable softening agents include aryl mercaptans such as xylol mercaptans, naphthyl beta mercaptan and alpha naphthyl mercaptan, aliphatic mercaptans, benzoyl peroxide and the like. The presence of the softening agent reduces the power required for the compounding mill, causes "bending" on the rolls in a much shorter time, permits of easy calendering and extruding, and, in general, greatly simplifies the processing treatment and improves the workability of the polymer.

According to the present invention the compounding with the softening agent is carried out in a continuous manner through a series of train operations including a dryer, an extruder, a friction mill and a sheeting mill. The plasticizing agent is continuously added to the polymer as it enters the extruder. This series of operations results in a high Mooney polymer being reduced to a value where it will be acceptable from a processability standpoint, i. e. a Mooney viscosity of 40-55.

In the usual method of plasticizing such polymers it has been the practice to add the plasticizing agent to open the roller mills and work the polymer until it has been reduced to the

desired plasticity. This, however, results in considerable loss of plasticizer by evaporation and decomposition and only a portion of the added plasticizer is effective. Furthermore, there is also danger that a small amount of residual plasticizer remains in the finished polymer causing breakdown in use.

The present invention therefore provides a new process for carrying out the plasticization of rubber-like materials with means for separating and recovering the plasticized polymer substantially without loss of any of the plasticizing agent.

Broadly the apparatus of the present invention comprises a plasticizing vessel in combination with an extruder followed by the usual mill. The plasticizing vessel contains screws forming a part of the extruding mechanism, with the screws operating directly in the plasticizable mixture. The plasticizing apparatus is preferably tightly closed with solid covers and is provided with supply lines for the delivery of the polymer and the plasticizing agent. The screws force the plasticized polymer through a die section which extrudes the polymer as a solid plug or blanket. The extruded polymer is preferably conveyed to a roller mill where the plasticization is continued in the open, and then conveyed to a second mill where it is cooled and stripped onto another conveyor. This conveyor leads to a cooling train and then to a cutter and stacker arrangement prior to packaging.

Referring now to Figure 1, a metered amount of polymer is removed from tunnel drier 10 as a porous blanket which is cut into strips about 6 in. in width (not shown) and carried by conveyor 11 to plasticizing zone 12 containing screws 13, where it is mixed with an aryl mercaptan or other plasticizer from supply tank 14 and rotameter 15, the amount of plasticizer depending on the original Mooney viscosity and temperatures of operation. The plasticizing vessel 12 operates at a temperature of 300° to 340° F. Screws 13 thoroughly mix the mercaptan with the polymer, softening it and conveying it to the discharge end of the vessel which is fitted with die plate 16, through which the polymer is forced as a sheet or blanket onto conveyor 17 to friction mill 18 operating at 300° to 350° F. where it is milled for ten minutes. From the friction mill it is carried by conveyor 19 to sheeting mill 20 operating at a temperature of 280° to 330° F. and then removed by conveyor 21 for packaging.

The proper control of the finishing operation above described is dependent upon certain factors. These factors are the concentration of plasticizing agent, temperature of operation, original Mooney viscosity, original average molecular weight and degree of unsaturation, and residence time on the mill. The importance of these factors is indicated in the following examples. Although the data do not show the original average molecular weight, the original Mooney viscosity affords a general indication of the average molecular weight.

#### Example 1

Four isobutylene-isoprene copolymers were selected to give samples with Mooney viscosity values of 50, 60, 70 and 80. These samples were plasticized on a laboratory mill in the presence of a range of aryl mercaptan concentrations. The mill load was maintained at 100 grams, and the mill setting was adjusted at a specific temperature so as to provide an active mill bank. The mill

temperature was increased between 100° and 300° F. in increments of 50° F. The plasticized samples were tested for Mooney viscosity, mill temperature, and concentration of mercaptan. To show the inter-relationship of the factors studied, these data are shown graphically in Figures 2 through 6.

In considering the limits of mercaptan concentration required for the operation of this process, the concentration of mercaptan as added to the polymer is not the effective mercaptan concentration. The amount of mercaptan residing in the polymer after 10 minutes milling period at 300° F. is approximately 30 per cent of that originally added. The remainder of the mercaptan originally added is lost by volatilization and/or decomposition. This condition is peculiar to open systems such as the mill used in these studies, and not for closed systems such as that represented by an extruder. For this reason, two sets of data are represented on each graph for a given temperature of operation. One set of data shows the relation between Mooney viscosity reduction and the mercaptan content originally added, while the other set shows the relation between Mooney viscosity reduction and the mercaptan content after 10 minutes hot milling at the specified temperature. To estimate the mercaptan requirements for a desired degree of plasticization, it will only be necessary to refer to the proper curve dependent on whether an open mill or an extruder system is to be employed.

It will be noted that the efficiency of plasticization (degree of plasticization achieved for increasing concentration of mercaptan) increases gradually as the temperature of milling increases. At a milling temperature of 250° F. the efficiency increases quite markedly over that obtained in the lower range of temperatures. The increase in efficiency at temperatures above 250° F. is small. It is concluded on the basis of these observations that a critical temperature with respect to plasticization efficiency exists in the approximate region of 250° F.

That this temperature is actually critical is more clearly shown from the following data on the slope of the mercaptan concentration curve for each 50° increment in temperature.

| 50  | Mill Temperature, °F. | Slope <sup>1</sup> |
|-----|-----------------------|--------------------|
| 100 |                       | 0.159              |
| 150 |                       | 0.214              |
| 200 |                       | 0.214              |
| 250 |                       | 0.425              |
| 300 |                       | 0.421              |

<sup>1</sup> Mooney viscosity reduction as a function of mercaptan concentration. These values are average values of the slope of the curves for polymers of original Mooney viscosity values of 50, 60, 70 and 80, the slope being determined from a plot of the logarithm of Mooney viscosity versus the logarithm of mercaptan concentration and being equal to the ratio

$$60 \quad \frac{\log V_A - \log V_B}{\log C_A - \log C_B}$$

wherein  $V_A$  and  $V_B$  are the ordinates (Mooney viscosity) of any two points A and B respectively, and  $C_A$  and  $C_B$  are the abscissas (mercaptan concentration) of the same two points.

65 It is apparent from these data that a given concentration of mercaptan becomes significantly more efficient at a mill temperature of 250° F.

The practical working rule to be based on this conclusion is that a temperature of 250° F. or above must be employed in plasticization work in order to insure constant plasticization action with a given mercaptan concentration.

70 These data also show the relation of the Mooney viscosity reduction to the concentration of mercaptan employed. The Mooney viscosity values of

the polymers decrease regularly as the logarithmic function of the concentration of mercaptan. From these data it is evident that for an optimum temperature of 300° F. and a polymer having an original Mooney viscosity between 55 and 80, the effective mercaptan necessary to reduce the viscosity to the usual specification of 50 is about 0.017-0.060% by weight of polymer. For polymers in the range of 55-60, the effective amount of mercaptan to be added is 0.017-0.021, for an original viscosity of 60-70 the amount of mercaptan is 0.020-0.033 and for an original viscosity of about 80 the amount of mercaptan is 0.033 to 0.06%.

It is also evident the original Mooney viscosity value of the polymer affects the plasticization. This effect seems to be limited to the fact that the higher the original Mooney viscosity value, the greater is the concentration of mercaptan required to achieve plasticization to a given point.

#### Example 2

A series of polymers of varying degrees of unsaturation was hot milled in the present of 0.2 per cent naphthyl-beta-mercaptop in order to show the effect of unsaturation on plasticization. The observations recorded in this experiment are shown below:

| Polymer Type                    | Original Mol. Wt. (a) | Unsaturation Mole % (b) | Mooney Viscosity (c) |             | Extrusion Minutes (a) | Extrusion Rate Grams/min. | Plasticizer (b) Concentration (c), per cent on Polymer | Mooney Vis., 1½ Min. at 100° C. |
|---------------------------------|-----------------------|-------------------------|----------------------|-------------|-----------------------|---------------------------|--------------------------------------------------------|---------------------------------|
|                                 |                       |                         | Original             | Plasticized |                       |                           |                                                        |                                 |
| Polyisobutylene                 | 157,000               | 0.26                    | 55                   | 59          | 0                     |                           | 0.0                                                    | 78                              |
| Isobutylene plus 0.5% isoprene  | 71,000                | 0.43                    | 77                   | 65          | 2                     | 54.5                      | 0.20                                                   | 53                              |
| Isobutylene plus 0.5% isoprene  | 72,000                | 0.50                    | 76                   | 72          | 4                     | 67.5                      | 0.14                                                   | 48                              |
| Isobutylene plus 0.5% isoprene  | 83,000                | 0.37                    | 70                   | 79          | 6                     | 71.0                      | 0.10                                                   | 49                              |
| Isobutylene plus 1.27% isoprene | 67,000                | 1.27                    | 79                   | 61          | 7.5                   | 63.0                      | 0.15                                                   | 55                              |
| Isobutylene plus 1.97% isoprene | 48,000                | 1.62                    | 77                   | 39          | 9                     | 67.5                      | 0.17                                                   | 60                              |
| Isobutylene plus 2.75% isoprene | 47,000                | 2.27                    | 75                   | 34          | 12                    | 70.5                      | 0.30                                                   | 41                              |
|                                 |                       |                         |                      |             | 13.5                  | 69.0                      | 0.15                                                   | 46                              |
|                                 |                       |                         |                      |             | 15                    | 74.5                      | 0.10                                                   | 53                              |
|                                 |                       |                         |                      |             | 16.5                  | 70.5                      | 0.18                                                   | 51                              |
|                                 |                       |                         |                      |             | 18                    | 73.5                      | 0.22                                                   | 44                              |
|                                 |                       |                         |                      |             | 19.5                  | 64.0                      | 0.20                                                   | 47                              |
|                                 |                       |                         |                      |             | 21                    | 64.0                      | 0.22                                                   | 46                              |
|                                 |                       |                         |                      |             | 22.5                  | 67.5                      | 0.21                                                   | 44                              |
|                                 |                       |                         |                      |             | 24                    | 61.5                      | 0.23                                                   | 48                              |
|                                 |                       |                         |                      |             | 25.5                  | 71.5                      | 0.15                                                   | 49                              |
|                                 |                       |                         |                      |             | 27                    | 69.5                      | 0.12                                                   | 53                              |
|                                 |                       |                         |                      |             | 30                    | 69.5                      | 0.15                                                   | 44                              |
|                                 |                       |                         |                      |             | 31.5                  | 71.5                      | 0.21                                                   | 48                              |

(a) Staudinger scale.

(b) Iodine chloride method.

(c) Determination made at 100° C., one minute warmup, and 1½ minutes under shear.

NOTE: The polymers were plasticized for 10 minutes on an open laboratory mill at 300° F. in the presence of 0.2% naphthyl-beta-mercaptop (0.06% effective).

The fact that the degree of plasticization obtainable under a given set of conditions is affected by the unsaturation of the polymer is clearly shown by the data recorded above. It will be noted that the degree of plasticization obtained increases as the unsaturation value of the polymers increases. It is quite apparent that in order to obtain any substantial reduction in viscosity, the unsaturation must be at least 1.27 mol per cent, preferably 1.62% as determined by the iodine chloride method. In view of this difference in response, it is imperative that in the chemical plasticization operation the degree of unsaturation of the polymer being plasticized must be kept relatively constant. If the degree of unsaturation of the polymers to be plasticized varies, then the mercaptan ratio must also be varied.

#### Example 3

To show the effect of plasticizing the polymer in an extruder, polymer and mercaptan were both fed into the hopper of a laboratory type extruder simultaneously. The extruder was operated at a temperature of 300° F. and a worm speed of 70 R. P. M. The extruder die con-

sisted of a 0.4 inch diameter die and a 0.3 inch diameter pin. The polymer employed was the type resulting from the polymerization of isobutylene with 2.5% isoprene having an original Mooney viscosity value of 78, when the test was conducted for 1½ minutes at 100° C. The mercaptan employed in this experiment was xylol mercaptan which is supplied commercially as a 36.5 weight per cent solution in a kerosene type solvent. The mercaptan solution was added from a burette. The extrusion experiment was continued for 30 minutes. The concentration of mercaptan on a polymer basis was calculated to give a reduction in Mooney viscosity from a value of 78 to 48. Since it was not known how much hot milling would be required subsequent to the extrusion operation, the extruded polymer was milled for 10 minutes after it had been extruded. The results of this continuous plasticization experiment are shown in the following table:

| Polymer Type                    | Original Mol. Wt. (a) | Unsaturation Mole % (b) | Mooney Viscosity (c) | Extrusion Minutes (a) | Extrusion Rate Grams/min. | Plasticizer (b) Concentration (c), per cent on Polymer | Mooney Vis., 1½ Min. at 100° C. |
|---------------------------------|-----------------------|-------------------------|----------------------|-----------------------|---------------------------|--------------------------------------------------------|---------------------------------|
| Polyisobutylene                 | 157,000               | 0.26                    | 55                   | 35                    | 0                         | 0.0                                                    | 78                              |
| Isobutylene plus 0.5% isoprene  | 71,000                | 0.43                    | 77                   | 35                    | 2                         | 0.20                                                   | 53                              |
| Isobutylene plus 0.5% isoprene  | 72,000                | 0.50                    | 76                   | 35                    | 4                         | 0.14                                                   | 48                              |
| Isobutylene plus 0.5% isoprene  | 83,000                | 0.37                    | 70                   | 35                    | 6                         | 0.10                                                   | 49                              |
| Isobutylene plus 1.27% isoprene | 67,000                | 1.27                    | 79                   | 40                    | 7.5                       | 0.15                                                   | 55                              |
| Isobutylene plus 1.97% isoprene | 48,000                | 1.62                    | 77                   | 40                    | 9                         | 0.17                                                   | 60                              |
| Isobutylene plus 2.75% isoprene | 47,000                | 2.27                    | 75                   | 40                    | 12                        | 0.30                                                   | 41                              |
|                                 |                       |                         |                      |                       | 13.5                      | 0.15                                                   | 46                              |
|                                 |                       |                         |                      |                       | 15                        | 0.10                                                   | 53                              |
|                                 |                       |                         |                      |                       | 16.5                      | 0.18                                                   | 51                              |
|                                 |                       |                         |                      |                       | 18                        | 0.22                                                   | 44                              |
|                                 |                       |                         |                      |                       | 19.5                      | 0.20                                                   | 47                              |
|                                 |                       |                         |                      |                       | 21                        | 0.22                                                   | 46                              |
|                                 |                       |                         |                      |                       | 22.5                      | 0.21                                                   | 44                              |
|                                 |                       |                         |                      |                       | 24                        | 0.23                                                   | 48                              |
|                                 |                       |                         |                      |                       | 25.5                      | 0.15                                                   | 49                              |
|                                 |                       |                         |                      |                       | 27                        | 0.12                                                   | 53                              |
|                                 |                       |                         |                      |                       | 30                        | 0.15                                                   | 44                              |
|                                 |                       |                         |                      |                       | 31.5                      | 0.21                                                   | 48                              |

(a) Extruder and mill operated at 300° F. After extrusion, the polymer was milled for 10 minutes at 300° F.

(b) Xylol mercaptan.

(c) The concentrations reported are those actually added to the polymer. The estimated active ingredient utilized in the plasticization is 30% of the amount added to the polymer.

The data show that mercaptan can be added to the polymer entering the extruder in a continuous manner sufficiently well controlled so as to provide a uniform reduction in the Mooney viscosity value of the polymer.

#### Example 4

To determine the minimum amount of time of hot milling required in the combined extruder-mill plasticization process described in Figure 1, a polymer of 78 Mooney viscosity value was extruded at 300° F. for various numbers of cycles and then hot milled for varying periods of time at 300° F. A concentration of 0.2 per cent (0.06 per cent effective) xylol mercaptan was added to the polymer on a cold mill prior to extrusion. The data recorded in this experiment are shown in Figure 7.

From these data it is apparent that the extruder operation itself contributes to the degree of plasticization obtained. The significant point to be noted in these data is that a single cycle through the extruder at 300° F. followed by 3 minutes milling at 300° F. is all that is required to reduce a polymer of 78 Mooney viscosity value to a point where it will be acceptable from a processability standpoint (a Mooney viscosity range of 40-55).

#### Example 5

A typical plasticization operation was carried

out in the continuous train operation described in Figure 1 using an extruder having a  $\frac{1}{4} \times 14$  in. orifice, at a temperature of 300° F. in the extruder and mill and in the presence of 0.06-0.09% (.018-.027% effective) of added mercaptan measured into the extruder hopper through a rotameter. In each case only enough mercaptan was added to give the desired results. The following results were obtained:

| Time, P. M. | Mooney Viscosity  |                  |             |                  |             |
|-------------|-------------------|------------------|-------------|------------------|-------------|
|             | Entering Extruder | Leaving Extruder | On Hot Mill | Finished Product | Special (a) |
| 3:30.....   | 62                | 49               | 53          | 49               | 50          |
| 4:00.....   | 60                | 45               | 48          | 50               | 47          |
| 4:30.....   | 61                | 51               | 50          | 49               | 47          |
| 5:00.....   | 63                | 54               | 53          | 51               | 51          |
| 5:30.....   | 62                | 55               | 54          | 52               | 50          |
| 6:00.....   | 63                | 50               | 51          | 51               | 49          |
| 6:30.....   | 67                | 55               | 51          | 50               | 51          |
| 7:00.....   | 67                | 53               | 50          | 53               | 48          |
| 7:30.....   | 68                | 53               | 55          | 56               | 46          |
| 8:00.....   | 59                | 52               | 50          | 50               | 47          |
| 8:30.....   | 58                | 46               | 48          | 46               | 46          |
| 9:00.....   | 59                | 44               | 48          | 45               | 41          |
| 9:30.....   | 58                | 46               | 49          | 47               | 47          |
| 10:00.....  | 55                | 47               | 47          | 47               | 47          |

(a) Finished product milled at 300° F. on a laboratory mill for 10 minutes. A decrease in Mooney viscosity value indicates the presence of residual active mercaptan.

These data show that it is possible to maintain the plasticity of the product within close limits by application of the continuous chemical plasticization process. Furthermore, the data from Fig. 6 indicates that for the plant operation the amount of mercaptan added to the extruder to reduce an original polymer having a Mooney viscosity value of between 50 and 80 to the specification value of 40-55 Mooney viscosity should be about 0.2 (0.06% effective) by weight of the polymer on the mill.

It may be noted that, while the process has been described only in connection with the plasticization of copolymers of isobutylene with isoprene, it is evident that the process is applicable to the processing of all types of rubber-like polymers, such copolymers of butadiene with styrene, acrylonitrile, etc., polychlorobutadiene polymers, polyethylene polymers, polymethacrylates, polyisobutylene, natural rubber, etc. However, the invention finds particular applicability in connection with those types of polymers having molecular weights above 15,000 Staudinger numbers and low unsaturation values as indicated by iodine numbers below 50.

Thus, by the method of the present invention, the processing of polymer material is greatly simplified and its plasticity prior to curing is improved without injury to its cured properties, by the use of a continuous plasticizing process employing a series of train operations.

Although the present invention has been described with a certain degree of particularity, it is understood that the present disclosure has been made only by way of example and that numerous changes in the details of operation may be resorted to without departing from the spirit and scope of the invention.

The nature and objects of the present invention having thus been described and illustrated, what is claimed as new and useful and desired to be secured by Letters Patent is:

1. A process for the continuous production of a high molecular weight, rubber-like copolymer product of a major proportion of a 2-methyl alkene-1 having a total of 4 to 6 carbon atoms per molecule and a minor proportion of a polyolefin

having 4 to 10 carbon atoms per molecule, said copolymer having an unsaturation which is equivalent to at least 1.27 mol percent of combined diolefin per mol of copolymer, and having a Mooney viscosity V within the range between 40 and 55, from a plasticizable copolymer having originally a known, varying Mooney viscosity  $V_0$  up to 80 and higher than V, which comprises continuously introducing the more viscous co-

10 polymer into a plasticizing zone maintained at a temperature between 250° F. and 340° F., simultaneously introducing into said zone an aryl mercaptan plasticizer at a rate which varies between 0.017 and 0.060 weight percent of effective mercaptan per copolymer, mechanically working the mixture of copolymer and plasticizer in the plasticizing zone, and continuously recovering the worked copolymer from the plasticizing zone.

15 2. A process for continuously preparing a rubber-like product characterized by a Mooney viscosity value of between 40 and 55 from a high molecular, rubber-like copolymer of a major proportion of isobutylene and a minor proportion of a diolefin having 4 to 6 carbon atoms per mole-

20 cule, said copolymer having an unsaturation value of at least 1.27 mol percent of combined diolefin per mol of copolymer, and also having a known, undesirably high and variable Mooney viscosity between 50 and 80, comprising continuously introducing the copolymer of known, varying viscosity into a plasticizing zone maintained between 250 and 340° F., and simultaneously introducing into said zone an aryl mercaptan at a rate which varies between 0.017 and 0.060% of effective mercaptan by weight of copolymer, mechanically working the mixture of copolymer and plasticizer, and continuously extruding the worked copolymer from the plasticizing zone.

25 3. A process for continuously preparing a rubber-like product of uniform viscosity of between 40 and 55 Mooney from a high molecular, rubber-like copolymer of a major proportion of isobutylene and minor proportion of isoprene, said copolymer being characterized by an unsaturation

30 value of between 1.27 and 2.27 mol percent of combined isoprene per mol of copolymer, and also being characterized by a known, undesirably high and varying Mooney viscosity between 50 and 80, comprising continuously introducing the copolymer of known, varying viscosity into a plasticizing zone maintained between 250° F. and 340° F., simultaneously introducing into said zone beta-naphthyl mercaptan at a rate which is varied from a lower limit of 0.017 weight percent of effective mercaptan by weight of introduced copolymer when said copolymer has an original Mooney viscosity of 50 to an upper limit of 0.060 weight percent of mercaptan when the introduced copolymer has an original Mooney

35 viscosity of 80, mechanically working the mixture of copolymer and plasticizer until the Mooney viscosity of the mixture is reduced to between 40 and 55, and continuously removing the plasticized product from the plasticizing zone.

40 4. A process for the continuous preparation of a rubber-like product having a Mooney viscosity within the limits of 40 and 55 from a high molecular, rubber-like copolymer of a major proportion of isobutylene and a minor proportion of isoprene, the said copolymer having an unsaturation value between 1.27 and 2.27 mol percent of combined isoprene per mol of copolymer and also having a known Mooney viscosity which varies during the processing period between 50 and 80, comprising continuously introducing said

copolymer of known, varying viscosity into an enclosed plasticizing zone maintained between 250 and 340° F., also continuously introducing into said plasticizing zone beta naphthyl mercaptan at a rate which is varied from a lower limit of 0.017 weight percent of mercaptan by weight of copolymer when the latter has an original viscosity of 50, to an upper limit of 0.060 weight percent of mercaptan when the introduced copolymer has an original Mooney viscosity of 80, thoroughly mixing the mercaptan with the copolymer to soften the latter, extruding the mixture from the plasticizing zone, conveying the extruded mixture to a milling zone maintained also at a temperature between 250 and 340° F., mechanically working the mixture in the milling zone until the Mooney viscosity of the mixture is reduced to a value within the range of 40 to 55,

5

10

15

and recovering the plasticized mixture from the milling zone.

5. A process according to claim 2 wherein the mercaptan plasticizer is xylyl mercaptan.

DONALD J. BUCKLEY.  
ALLEN L. CHANEY.

## REFERENCES CITED

The following references are of record in the file of this patent:

## UNITED STATES PATENTS

| Number    | Name       | Date          |
|-----------|------------|---------------|
| 1,990,555 | Loomis     | Feb. 12, 1935 |
| 2,021,961 | MacFarlane | Nov. 26, 1935 |
| 2,319,859 | Hale       | May 25, 1943  |
| 2,333,403 | Youker     | Nov. 2, 1943  |
| 2,333,786 | Hessen     | Nov. 9, 1943  |